# EUROPEAN PATENT SPECIFICATION

(11) **EP 0 984 101 B1**
(45) Date of publication and mention of the grant of the patent: **14.07.2004**
(21) Application number: 99660129.0
(22) Date of filing: 20.08.1999
(51) Int. Cl.: D21H 17/18

(54) **A sizing composition usable for the neutral sizing of paper or board, and a process for the manufacture of paper or board**
Leimungsmittel verwendbar für die neutrale Leimung von Papier oder Karton und Verfahren für die Herstellung von Papier oder Karton
Composition de collage utilisable pour le collage neutre de papier ou de carton et procédé pour sa fabrication

(30) Priority: 04.09.1998 FI 981893
(43) Date of publication of application: 08.03.2000
(73) Proprietor: Kemira Oyj, 00180 Helsinki (FI)
(72) Inventor: Juppo, Ari, 65230 Vaasa (FI); Paren, Aarto, 65230 Vaasa (FI)
(74) Representative: Svensson, Johan Henrik

(56) References cited:
- EP-A- 0 073 872
- WO-A-94/13883

## Description

The present invention relates to a sizing composition usable for the neutral sizing of paper or board. The invention additionally relates to a process for the manufacture of paper or board.

At a neutral pH, alkyl ketene dimer (AKD) or alkenyl succinic acid anhydride (ASA) is commonly used as a size in order to enhance the water repellence (hydrophobicity) of paper or board. Both of these molecules are deemed to react with cellulose fiber. The reaction occurs most rapidly in particular in alkaline or slightly basic conditions. In paper making, AKD and ASA are added to an aqueous dispersion which contains fiber and additives (e.g. fillers, retention agents, anti-foaming agents, pH control agents), and from which an effort is made to separate the solids onto the wire as effectively as possible, i.e. the aim is as high a retention as possible. The water used for the dispersion is commonly circulation water and pure raw water added to it, in which case the water used for the dispersing usually contains, for example, approx. 200 ppm of alkaline earth metals: calcium and magnesium ions.

WO-A-94/13883 discloses the use of a neutral sizing agent like e.g. ASA or AKD, for sizing paper or board.

It is commonly known that pulps which contain calcium carbonate, which is used for increasing the brightness of paper, consume more hydrophobification chemicals than do pulps without carbonate.

Carboxyl groups on the surface of cellulose generate a negative charge in the fibers. The magnitude of the charge depends on the surrounding pH. In alkaline conditions the carboxyl group becomes protolyzed, and therefore the quantity of negative charges increases.

In general the sizes used for purposes of hydrophobification are prepared by emulsifying the water-repellent substance in a cationically charged starch. The starch surrounds the water-insoluble hydrophobification agent, whereupon a dispersion evenly distributed in the water is formed. Owing to the starch the dispersion particles are cationic. They tend to adhere to negatively charged surfaces, for example cellulose fibers.

In particular in hard waters, bivalent alkaline earth metal ions, such as Ca²⁺ ions, and also other multivalent ions, neutralize the carboxyl groups of cellulose fibers, and consequently the negative charge of the fibers respectively decreases. Since it has been conceived that a size particle formulated using a cationic starch attaches to the fiber surface by means of charges, the presence of surface charges both in the size particle and the fiber is important in terms of retention. Ca²⁻ ions neutralize the surface charge, and consequently the retention of cationic size particles weakens. Likewise, the adherence of cationic retention agents to fiber also depends on the surface charge of the fiber.

By the use of chelating and sequestering chemicals, by means of which the quantity of free ions in waters can be lowered, it is also possible to decrease the number of Ca²⁺ ions on fiber surfaces and to create free anionic groups to enhance retention. However, if these complexing agents were used directly, for example, in the circulation waters of the paper machine, their use would be relatively high and would cause problems in the rest of the operation of the machine.

It has been observed, surprisingly, that paper hydrophobification by using AKD- and ASA-based chemicals can be improved when small amounts of agents which form complexes with metals are added to their formulations or are dosed together with them. Thus, by means of the agents added to the size, the complexing of the cations in the fiber is brought close to the size particles, whereby the retention of the size is improved, while the concentration of complexing agents in the circulation waters of the paper machine can, nevertheless, be maintained low.

Since, for example, calcium carbonate is a commonly used filler in paper making, the use of complexing agents for chelating all of the calcium is not sensible, since this would lead to the dissolving of the calcium carbonate. What is inventive here is specifically the fact that it has been observed, surprisingly, that a very small dose of complexing agents in the size formulation considerably improves sizing. In terms of the performance of the invention it is required that the complexing agent sufficiently rapidly forms sufficiently stable complexes with the metal cations which are present in the paper machine and possibly have a deleterious effect on AKD sizing. It is essential for the performance of the invention that a suitable quantity of complexing agents is added to the size formulation.

According to the invention, there is thus provided for the neutral sizing of paper or board a sizing composition containing
(i) a size capable of reacting with cellulose, said size being an alkyl ketene dimer (AKD) or an alkenyl succinic acid anhydride (ASA), and
(ii) an organic complexing agent in an amount of 0.1-20% by weight of the amount of the size.

The term chelating agent is also used for complexing agents.

Suitable complexing agents which can be used in accordance with the invention include
a) aminopolycarboxylic acids
b) N-bis- or tris-[(1,2-dicarboxylethoxy)ethyl]amines and
c) phosphonic acids.

The complexing agents cited above may be in the form of an acid or a salt. Suitable salts include alkali metal salts and ammonium salt. Sodium and potassium salts are preferred salts.

Preferred complexing agents of group a) include aminopolycarboxylic acids having the following general Formula I. where
A is -CH₂COOH,
B is -CH₂COOH or -CH₂CH₂OH,
x is 0-6, preferably 0-3,
y is 0-6, preferably 0-2,
a is 2-10, preferably 2-4, and
b is 2-10, preferably 2-6.

Especially preferable compounds according to Formula I include ethylene diamine tetra-acetic acid, i.e. EDTA (B=A, x=0, b=2 and y=1), diethylene triamine penta-acetic acid, i.e. DTPA (B=A, x=1, a=2, b=2 and y=1), and
nitrilotriacetic acid, i.e. NTA (B=A, x=0 and y=0).

Preferred complexing agents of group b) include N-bis- or tris-[(1,2-dicarboxylethoxy)ethyl]amines having the general Formula II where
R is hydrogen,
an alkyl group having 1-30 carbon atoms,
an alkyl group having 1-30 carbon atoms and additionally 1-10 carboxylic acid groups,
an alkyl group having 1-30 carbon atoms and additionally 1-10 carboxylic acid ester groups,
a (poly)ethoxylated hydrocarbon group having 1-20 ethoxyl groups, or
a carboxylic acid amide group having 1-30 carbon atoms, in which case the N-R bond is an amide bond.

Especially preferable complexing agents in Formula II include the following compounds according to Formulae A, B and C:
- A=: N-bis[(1,2-dicarboxylethoxy)ethyl]amine (hereinafter the acronym BCEEA will be used)
- B=: N-bis[(1,2-dicarboxylethoxy)ethyl]aspartic acid (hereinafter the acronym BCEEAA will be used)
- C=: N-tris[(1,2-dicarboxylethoxy)ethyl]amine (hereinafter the acronym TCEEA will be used)

These complexing agents A, B and C and their preparation have been described in patent application FI-962261. It is also possible to use mixtures of compounds A and B.

Preferred complexing agents of group c include phosphonic acids having the general Formula III where
R₁ is hydrogen, a lower alkyl such as -CH₃ or -(CH₂)ₙ-CH₃, an amino group -NH₂, hydroxy methyl -CH₂OH, a lower carboxylic acid group -(CH₂)ₙ-COOH, a lower alkyl phosphonic acid group -(CH₂)ₙ-PO₃H₂, or a group having the formula
R₂ is hydrogen, hydroxyl -OH, a phosphonic acid group -PO₃H₂, a lower carboxylic acid group -(CH₂)ₙ-COOH or a group having the formula tai
R₃ is hydrogen, hydroxyl -OH, an amino group -NH₂, a lower alkyl such as -CH₃ or -(CH₂)ₙ-CH₃, a lower carboxylic acid group -(CH₂)ₙ-COOH or a group having the formula

   -NH-(CH₂)ₙ-PO₃H₂

   -NH-CH₂-COOH

   or
n is 0-6, preferably 0-3.

In the sizing composition according to the invention, the amount of the organic complexing agent is 0.1-20 % by weight, and especially preferably 0.2-3 % by weight, of the amount of the size.

The sizing composition according to the invention is preferably in the form of a dispersion, in which case it additionally contains a dispersion stabilizing agent.

The stabilizing agents of AKD dispersions include starch, cationic starch and other polymers, such as polyethylene imine, polyepiamine, a polydiethyl diallyl or dicyandiamide compound, polyacrylamide or polyacrylic acid, or salts of these.

For the stabilization of ASA dispersions it is possible to use, for example, starch or other polymers, such as water-soluble cellulose derivatives, e.g. hydroxyethyl or hydroxypropyl, methyl hydroxypropyl ethyl hydroxyethyl cellulose, carboxymethyl cellulose, gelatin, guar gum, xanthan gum or polyvinyl alcohol.

In the sizing composition according to the invention the amount of complexing agent may be 0.2-20 % by weight, preferably 0.2-10 % by weight, and especially preferably 1-5 % by weight, of the amount of the stabilizing agent.

According to the invention there is also provided a process for the manufacture of paper or board by neutral sizing by using a size capable of reacting with cellulose, said size being an alkyl ketene dimer (AKD) or an alkenyl succinic acid anhydride (ASA), the process being characterized in that an organic complexing agent defined above is incorporated into the size in an amount of 0.1-20% by weight of the amount of the size.

The invention additionally relates to the use of the sizing composition defined above for the neutral sizing of paper or board.

When the sizing composition or sizing formulation according to the invention contains starch, the complexing agent binds to the starch layer, from which it detaches in dilution and forms a complex with Ca²⁺ ions. When the complexing ion detaches from a fiber, the fiber becomes more anionic and the size particle adheres to the fiber. It is known that the equilibrium constant of cellulose fiber with respect to the complexing of Ca²⁺ ions is approx. 3. On the one hand, this shows that cellulose binds ions out of the circulation water and, on the other hand, this requires that the equilibrium constant of the additive which complexes Ca²⁺ ions must be higher than that of cellulose, as for example the constants of the substances mentioned above are approx. 10.

The sizing composition works in particular in pulps which are made in hard waters and in machines the retention of which is otherwise poor.

It is a common view that the hydrophobicity of paper produced by AKD sizing develops slowly. Rapid sizing is required in particular in the manufacture of base paper for coating. A considerable improvement can be achieved by using the composition according to the present invention.

The performance of the invention is not affected by the other chemicals, such as starch and calcium carbonate, used in the making of the paper, or by the quality of the pulp. Also, the order in which the chemicals are added in the paper machine or the other running parameters of the paper machine do not affect the performance of the invention.

The amount of complexing agent used in the sizing formulation may be 0.1-20 % by weight of the amount of AKD or ASA and 0.2-20 % by weight of the total amount of starch or other polymer stabilizing the formulation. These compounds can be used as such in acid form or in the form of their alkali or ammonium salts. If the agent is used in the form of a salt thereof, the cation of the said salt does not have a substantial effect on the performance of the invention.

Present-day AKD emulsions are physically stable and usable for several weeks. The concentration of AKD in the products may be 0.5-30 % by weight. Various starches are commonly used for the formulation of AKD. They are generally cationated either with quaternary amines, in which case the starch retains its cationic charge also in alkaline conditions, or with primary, secondary or tertiary amines, the charge of which is dependent on the pH. The amount of starch may be 0.1-10 times the proportion AKD. For the dispersing of AKD wax there are generally used various anionic chemicals, such as lignosulfonates, aliphatic or aromatic sulfonates, nonionic surfactants such as fatty acid or fatty alcohol ethoxylates, or cationic surfactants such as fatty acid amines or imidazolines. For the stabilizing of an AKD dispersion it is also possible to use polymers, such as polyethylene imine, polyepiamine, polydimethyl diallyl or dicyandiamide compounds, polyacrylamide or polyacrylic acid and its salts. It is commonly known that the amount of stabilizing chemicals is 1-200 % by weight of the amount of AKD. By the use of polymers it is possible not only to improve the stability of the product but also to affect the performance of the product in paper or board. The adding of stabilizing chemicals is prior art commonly used in the formulation of AKD products.

ASA is dispersed at the paper or board mill by using apparatus installed for this purpose. The prepared dispersion is run immediately to the paper or board machine. To facilitate the preparation of an ASA dispersion, there is usually added to the product a surfactant, such as dioctyl sulfosuccinate, octyl phenoxy polyethoxy ethanol, and polyethylene oxy dinonyl phenyl phosphate, polyethylene oxy sorbitane trioleate.

In general, at the preparation stage it is possible to use as stabilizing agents for liquid ASA dispersions starch or other polymers, such as water-soluble cellulose derivatives, e.g. hydroxy ethyl and hydroxy propyl, methyl hydroxy propyl and ethyl hydroxy ethyl cellulose, carboxy methyl cellulose, or gelatin, guar gum. xanthan gum, polyvinyl alcohol, etc. The drop size of the dispersion is in general on average 0.2-3 µm. The complexing agents can be added to ASA-based commonly known compositions.

The sizing composition according to the invention is suitable for use for chemical pulps, mechanical pulps, chemimechanical pulps, and mixtures of these.

The performance of the compositions which are the object of the present invention is illustrated with the following examples. The percentages are percentages by weight, unless otherwise indicated.

### Example 1

The change in the surface charge of fiber under the effect of a complexing agent was studies as follows.

A mixture of pine and birch sulfate pulps at a ratio of 50:50 was dispersed in ion exchange water and was ground to a Schopper number of 20 °. The pulp was filtered and redispersed to a consistency of 1 % a) in ion exchange water and b) in ion exchange water which contained 0.1 % DTPA as an Na salt. The pulps were stirred for approx. 1 hour. The pulps were washed with ion exchange water at pH 7. The charge of the fiber was determined using polydiallyl dimethyl ammonium chloride and its back titration with a Na salt of polyethylene sulfonate by a Mütek apparatus.

| | | |
|---|---|---|
| a. | Charge of pulp after wash | anionic 3.8 µequiv/g of pulp |
| b. | Charge of pulp after DTPA and wash | anionic 5.6 µequiv/g of pulp |

### Example 2

The effect of a complexing agent on the charge of an AKD size formulation was studied using a Mütek apparatus. To an AKD dispersion stabilized with cationic starch there was added the active ingredient of Complexing Agent 1 and Complexing Agent 2 in an amount of 6 % calculated from the amount of starch. The cationic charge was determined by titration with an Na salt of polyethylene sulfonate at pH 3.5. In this example and the examples presented hereinafter, Complexing Agent 1 contains BCEEA and BCEEAA at a molar ratio of 2:3 and Complexing Agent 2 is TCEEA.

| **Test** | **Charge (µequiv/g of product)** **pH 3.5** | **Charge (µequiv/g)** **pH 8** |
|---|---|---|
| No complexing agent | cationic 3.3 | anionic 2.8 |
| Complexing Agent 1 | cationic 2.7 | anionic 3.3 |
| Complexing Agent 2 | cationic 2.2 | |

### Example 3

In this example there was used a pulp the composition of which was 40 % chemical birch pulp, 40 % chemical pine pulp and as the filler 20 % calcium carbonate and pulp starch 5 kg/t. A dispersion of AKD was prepared in a 2 % starch, the concentrations of Complexing Agents 1 and 2 in the dispersion being 0.6 % of the amount of AKD. The AKD dose used was 1 kg/t, in which case the amount of active ingredient forming the complex was 6 g/t. Test sheets having a grammage of 80 g/m² were prepared from the pulp according to the instructions by Scan-C 26:76. Cobb 60 min was determined from the sheets immediately and after 10 min of curing at 105 °C. The Cobb 60 values lowered even if the total retentions in the sheets were almost 100 %. Cobb values describe the water absorption of the paper, and they mean the amount of water which the paper absorbs within a certain time (g/m²). The lower the Cobb value, the better the sizing result.

**Table 1**

| **Laboratory test** | | | |
|---|---|---|---|
| | **Normal** | **Compl. agent 1** | **Compl. agent 2** |
| Cobb 60 unmatured | 34.2 | 28 | 27.9 |
| Cobb 60 matured | 27.6 | 25.3 | 25.8 |

### Example 4

The pulp used in the pilot machine was 35 % chemical pine pulp and 65 % chemical birch pulp. The filler used was calcium carbonate 23 % of the dry pulp. At a speed of 80 m/min of the pilot machine a paper was run the grammage of which was 70 g/m². The rate of AKD used was 1 kg/t. The AKD size contained Complexing Agent 1 in an amount of 0.3 % of the amount of AKD. Although the total retentions of the pilot machine were good, in the product containing the complexing agent the uncured immediate Cobb 60 (g/m²) was clearly lower than in the corresponding product without a complexing agent.

**Table 2**

| **Pilot machine** | | |
|---|---|---|
| | **Normal** | **Complexing agent 1** |
| Total retention (%) | 95.2 | 95.0 |
| Cobb 60 (g/m²) immediately, uncured | 20.5 | 16.9 |

## Claims

1. A sizing composition usable for the neutral sizing of paper or board, the composition containing
(i) a size capable of reacting with cellulose, said size being an alkyl ketene dimer (AKD) or an alkenyl succinic acid anhydride (ASA), and
(ii) an organic complexing agent in an amount of 0.1-20 % by weight of the amount of the size.

2. A sizing composition according to Claim 1, **characterized in that** the organic complexing agent is a) aminopolycarboxylic acid, b) N-bis- or tris-[(1,2-dicarboxylethoxy)ethyl]amine or c) phosphonic acid.

3. A sizing composition according to Claim 2, **characterized in that** the organic complexing agent of group a) is diethylene triamine penta-acetic acid (DTPA), ethylene diamine tetra-acetic acid (EDTA) or nitrilotriacetic acid (NTA), or a salt thereof or a mixture thereof, and the organic complexing agent of group b) is N-bis[(1,2-dicarboxylethoxy)ethyl]amine (BCEEA), N-bis[(1,2-dicarboxylethoxy)ethyl]aspartic acid (BCEEAA) or N-tris[(l,2-dicarboxylethoxy)ethyl]amine (TCEEA), or a salt thereof or a mixture thereof.

4. A sizing composition according to any of the above claims, **characterized in that** the amount of the organic complexing agent is 0.2-3 % by weight of the amount of the size.

5. A sizing composition according to any of the above claims, **characterized in that** it is in the form of a dispersion and additionally contains a dispersion stabilizing agent.

6. A sizing composition according to Claim 5, **characterized in that** the stabilizing agent is a starch or some other polymer.

7. A sizing composition according to Claim 5 or 6, **characterized in that** the amount of the organic complexing agent is 0.2-20 % by weight, preferably 0.2-10 % by weight and especially preferably 1-5 % by weight of the amount of stabilizing agent.

8. Use of a sizing composition defined in any of Claims 1-7 for the neutral sizing of paper or board.

9. A process for the manufacture of paper or board by neutral sizing by using a size capable of reacting with cellulose, said size being an alkyl ketene dimer (AKD) or an alkenyl succinic acid anhydride (ASA), **characterized in that** an organic complexing agent is incorporated into the size in an amount of 0.1-20 % by weight of the amount of the size.

10. A process according to Claim 9, **characterized in that** a sizing composition defined in any of Claims 1-7 is used for the sizing.

## Patentansprüche

1. Leimzusammensetzung, verwendbar für die neutrale Leimung von Papier oder Karton, wobei die Zusammensetzung enthält:
(i) einen Leim, der in der Lage ist, mit Cellulose zu reagieren, wobei der Leim ein Alkylketendimer (AKD) oder ein Alkenylsuccinsäureanhydrid (ASA) ist, und
(ii) einen organischen Komplexbildner in einer Menge von 0,1-20 Gew.-% der Leimmenge.

2. Leimzusammensetzung nach Anspruch 1, **dadurch gekennzeichnet, dass** der organische Komplexbildner a) Aminopolycarbonsäure, b) N-bis- oder -tris-[(1,2-dicarboxylethoxy)-ethyl]amin oder c) Phosphonsäure ist.

3. Leimzusammensetzung nach Anspruch 2, **dadurch gekennzeichnet, dass** der organische Komplexbildner der Gruppe a) Diethylentriaminpentaessigsäure (DTPA), Ethylendiamintetraessigsäure (EDTA) oder Nitrilotriessigsäure (NTA) oder ein Salz oder eine Mischung davon ist und der organische Komplexbildner der Gruppe b) N-bis[(1,2-dicarboxylethoxy)-ethyl]amin (BCEEA), N-bis[(1,2-dicarboxylethoxy)ethyl]-asparaginsäure (BCEEAA) oder N-tris[(1,2-dicarboxylethoxy)-ethyl]amin (TCEEA) oder ein Salz oder eine Mischung davon ist.

4. Leimzusammensetzung nach einem der vorangehenden Ansprüche, **dadurch gekennzeichnet, dass** die Menge des organischen Komplexbildners 0,2-3 Gew.-% der Leimmenge beträgt.

5. Leimzusammensetzung nach einem der vorangehenden Ansprüche, **dadurch gekennzeichnet, dass** diese in Form einer Dispersion vorliegt und außerdem ein Dispersionsstabilisierungsmittel enthält.

6. Leimzusammensetzung nach Anspruch 5, **dadurch gekennzeichnet, dass** das Stabilisierungsmittel eine Stärke oder ein anderes Polymer ist.

7. Leimzusammensetzung nach Anspruch 5 oder 6, **dadurch gekennzeichnet, dass** die Menge des organischen Komplexbildners 0,2-20 Gew.-%, vorzugsweise 0,2-10 Gew.-% und besonders bevorzugt 1-5 Gew.-%, der Menge des Stabilisierungsmittels beträgt.

8. Verwendung einer Leimzusammensetzung nach einem der Ansprüche 1-7 zur neutralen Leimung von Papier oder Karton.

9. Verfahren zur Herstellung von Papier oder Karton durch neutrale Leimung unter Verwendung eines Leims, der in der Lage ist, mit Cellulose zu reagieren, wobei der Leim ein Alkylketendimer (AKD) oder ein Alkenylsuccinsäureanhydrid (ASA) ist, **dadurch gekennzeichnet, dass** ein organischer Komplexbildner in einer Menge von 0,1-20 Gew.-% der Leimmenge in den Leim eingearbeitet ist.

10. Verfahren nach Anspruch 9, **dadurch gekennzeichnet, dass** die in einem der Ansprüche 1-7 definierte Leimzusammensetzung zum Leimen verwendet wird.

## Revendications

1. Composition de collage utilisable pour le collage neutre de papier ou de carton, la composition contenant
(i) une colle capable de réagir avec la cellulose, ladite colle étant un dimère alkylcétène (AKD) ou un anhydride d'acide alcényl succinique (ASA), et
(ii) un agent complexant organique en une quantité de 0,1 à 20 % en poids par rapport à la quantité de la colle.

2. Composition de collage selon la revendication 1, **caractérisée en ce que** l'agent complexant organique est a) un acide aminopolycarboxylique, b) une N-bis- ou tris[(1,2-dicarboxyléthoxy)éthyl]amine ou c) un acide phosphonique.

3. Composition de collage selon la revendication 2, **caractérisée en ce que** l'agent complexant organique du groupe a) est l'acide diéthylènetriamine penta-acétique (DTPA), l'acide éthylènediamine tétra-acétique (EDTA) ou l'acide nitrilotriacétique (NTA), ou un sel de ceux-ci ou un mélange de ceux-ci, et l'agent complexant organique du groupe b) est la N-bis[(1,2-dicarboxyléthoxy)éthyl]amine (BCEEA), l'acide N-bis[(1,2-dicarboxyléthoxy)éthyl]aspartique (BCEEAA) ou la N-tris[(1,2-dicarboxyléthoxy)éthyl]amine (TCEEA), ou un sel de ceux-ci ou un mélange de ceux-ci.

4. Composition de collage selon l'une quelconque des revendications précédentes, **caractérisée en ce que** la quantité de l'agent complexant organique est de 0,2 à 3 % en poids par rapport à la quantité de la colle.

5. Composition de collage selon l'une quelconque des revendications précédentes, **caractérisée en ce qu'**elle est sous la forme d'une dispersion et contient en outre un agent stabilisant la dispersion.

6. Composition de collage selon la revendication 5, **caractérisée en ce que** l'agent stabilisant est un amidon ou un certain autre polymère.

7. Composition de collage selon la revendication 5 ou 6, **caractérisée en ce que** la quantité de l'agent complexant organique est de 0,2 à 20 % en poids, de préférence de 0,2 à 10 % en poids et de manière spécialement préférée de 1 à 5 % en poids, par rapport à la quantité de l'agent stabilisant.

8. Utilisation d'une composition de collage définie selon l'une quelconque des revendications 1 à 7 pour le collage neutre de papier ou de carton.

9. Procédé de fabrication de papier ou de carton par collage neutre en utilisant une colle capable de réagir avec la cellulose, ladite colle étant un dimère alkylcétène (AKD) ou un anhydride d'acide alcényl succinique (ASA), **caractérisé en ce qu'**un agent complexant organique est incorporé dans la colle en une quantité de 0,1 à 20 % en poids par rapport à la quantité de la colle.

10. Procédé selon la revendication 9, **caractérisé en ce qu'**une composition de collage définie dans l'une quelconque des revendications 1 à 7 est utilisée pour le collage.
